

# UNITED STATES PATENT OFFICE.

JOSEPH PLANTE, OF LEVIS, QUEBEC, CANADA.

## LUBRICATING COMPOSITION.

SPECIFICATION forming part of Letters Patent No. 357,227, dated February 8, 1887.

Application filed June 7, 1886. Serial No. 204,346. (No specimens.)

*To all whom it may concern:*

Be it known that I, JOSEPH PLANTE, of the town of Levis, Province of Quebec, Dominion of Canada, have invented a new and Improved Lubricating Composition, of which the following is a full, clear, and exact description.

My invention consists in a composition of matter for lubricating the axles of railroad-cars and for other lubricating purposes, the same being made up of powdered sulphur, peat, (black earth taken from the bog,) and oil, substantially as hereinafter described. Thus, to prepare this composition, I take in the proportion of about three pounds of powdered sulphur and mix it thoroughly with a bushel of peat, (more or less,) and add to the whole enough of machinery or other suitable oil—say eight gallons, more or less—to make of the mass, when the ingredients are stirred or 20 worked together, a thick paste. The proportion of oil, however, may vary considerably, according to the quality or description of it.

In using this composition for lubricating car-axles, for which it is mainly intended, the

peat advantageously replaces the cotton-waste 25 saturated with oil, which has heretofore been used for such purpose, and which not infrequently becomes so dry that it takes fire, whereas the peat will always remain mixed with the oil. Furthermore, if, on account of the 30 bad or heated condition of the axles or the boxes in which they run, the oil should take fire, the sulphurous acid formed by the combustion of the sulphur in the composition would speedily extinguish the fire. 35

Having thus fully described my invention, I claim as new and desire to secure by Letters Patent—

The herein-described composition of matter to be used for lubricating car-axles and for 40 other lubricating purposes, consisting of powdered sulphur, peat, and oil, substantially as and in the proportions specified.

JOSEPH PLANTE.

Witnesses:

MARCEL BOURGET,  
ISIDORE BELLEAU.